

H. S. LEWIS,  
COMPOSITE SHEET,  
APPLICATION FILED OCT. 20, 1919.

1,374,931.

Patented Apr. 19, 1921.

*Fig. 1.*



*Fig. 2.*



*Fig. 3.*



*Fig. 4.*



*Inventor  
Harry S. Lewis  
By Dr. Wilson Thompson  
Attorneys*

# UNITED STATES PATENT OFFICE.

HARRY S. LEWIS, OF BEAVER FALLS, NEW YORK.

## COMPOSITE SHEET.

1,374,931.

Specification of Letters Patent. Patented Apr. 19, 1921.

Application filed October 20, 1919. Serial No. 331,965.

To all whom it may concern:

Be it known that I, HARRY S. LEWIS, of Beaver Falls, in the county of Lewis, in the State of New York, have invented new and useful Improvements in Composite Sheets, of which the following, taken in connection with the accompanying drawings, is a full, clear, and exact description.

This invention relates to certain improvements in a composite sheet, capable of use for various purposes, but peculiarly designed and adapted for use as wall board.

The manufacture of wall board, as practised today, consists of building up, by the use of suitable adhesive, two or more plies of so-called wood pulp board manufactured from either ground wood pulp or from so-called paper stock board manufactured from waste papers, each ply being usually from .030 to .055 of an inch in thickness according to the number of plies desired for a certain desired thickness of the finished product, such product being usually from  $\frac{1}{16}$  to  $\frac{1}{4}$  of an inch thick.

Some grades of wall board are at present made entirely of board manufactured from ground wood pulp made from soft wood, such as spruce, balsam, hemlock, pine and poplar wood, while other manufacturers, to reduce the cost of production, use in the finished product center plies of board manufactured from old paper stock, which board commands much lower price in the market than that manufactured direct from the ground wood pulp, but the combined or finished board frequently lacks the rigidity and strength of the wall board manufactured from all fresh ground wood pulp.

Rigidity is the characteristic of greatest importance in connection with the product known as wall board and I have experimented extensively in an effort to produce a wall board of greater rigidity and strength as compared with the commercial wall board made today. My experiments have lead to a development quite remote from the present day manufacture of wall board and to the use of material heretofore considered impractical for that purpose, viz: the use of ground wood made from hard wood, such as beech, birch, maple, elm, chestnut, oak, etc., adequately steamed or boiled preliminary to grinding.

My early experiments demonstrated that

when hard wood was ground in the usual manner of grinding soft wood for the production of wood pulp, a product was obtained which was of very short fiber amounting to practically a wood flour, having very little strength, impractical for handling on a paper machine without admixture of other stock and commercially useless for the purpose at hand.

I have found, however, that if hard wood is properly and adequately steamed or boiled prior to grinding in the usual manner of grinding wood pulp, that a wood pulp is produced which when manufactured into board has the desired characteristic of unusual rigidity and strength.

Therefore, in the process of manufacturing wood pulp from hard wood, the wood is subjected to steaming and boiling preliminary to grinding and purely as illustrative of a suitable operation of that character the wood in a closed chamber may be subjected to the action of steam under pressure as, for instance, fifty pounds for a period of eighteen hours. It is then ground and formed into single ply in the usual manner of treating soft wood pulp.

The composite wall board is then built up of any desired number of plies or laminations of board consisting of or comprising wood pulp manufactured from hard wood. Or perhaps preferably the center plies may be formed of such board manufactured from wood pulp produced from hard wood and the outer or facing plies or laminations may be formed of the ordinary commercial wood pulp board manufactured from soft woods so that the composite board has a substantially white or grayish-white surface color characteristic of natural wood pulp manufactured from the soft woods and the center plies or laminations are of the brown or dark brown color found characteristic of wood pulp produced by grinding hard wood after steaming or boiling.

The advantages of this are at least two-fold:

First, the resultant product has a materially increased rigidity and strength, and

Second, the product can be produced at a much cheaper cost by reason of the availability and the relatively low price of hard wood for the manufacture of wood pulp.

I, therefore, claim as new and original,

the manufacture of a composite or built-up sheet suitable for wall board or other purpose, the center plies of which, or all or any of the plies of which, consist of or contain a 5 desired percentage of pulp made from the woods known as hard, after such woods have been steamed or boiled as hereinbefore described, thereby increasing the rigidity and strength and decreasing the cost of production of the completed board as compared 10 with the wall board of commerce as made today.

In the manufacture of the single plies of board which are afterward laminated or 15 built up into the plural ply or finished wall board, a single ply sheet or web is built up on the so-called board machine in two or more layers by the use of two or more cylinders, these layers adhering to each other be- 20 cause of the pressure exerted upon the web while it is still in a moist state. In this manner it is possible to manufacture a web or sheet of single ply board for use as the two outside plies, sheets or laminations for 25 the finished composite board, with as many cylinders as desired running on the pulp produced from steamed or boiled hard wood and with one or more cylinders running on 30 pulp of other character, such as that produced from soft woods, so that the finished single ply sheet may consist of any desired number of layers formed from wood pulp manufactured from hard wood and any desired number of layers formed from wood 35 pulp manufactured from soft wood or other material and the finished single ply sheet may, therefore, have any desired shade or color upon either or both sides while the center or either or both sides may consist 40 entirely of board containing any percentage desired of the pulp made from the steamed or boiled hard wood of characteristic brown color.

In the drawings, I have illustrated various 45 forms that my invention may take.

Figure 1 is an elevation of a sample of wall board manufactured in accordance with my invention.

Fig. 2 is a vertical section of the same.

50 Figs. 3 and 4 are vertical sections of modified constructions of wall board made in accordance with my invention.

In Fig. 1, I have shown a wall board consisting of five plies, laminations, or sheets, 55 numbered 1, 2, 3, 4 and 5, respectively. The plies 1 and 5 are formed of the usual board manufactured from wood pulp produced from soft wood or other material and are of the grayish-white color characteristic of 60 board so manufactured, while the three inner plies, numbered 2, 3 and 4, are of the brown color found characteristic of board manufactured from pulp produced from hard wood after the same has been steamed or 65 boiled. The five sheets or plies are united

by any suitable adhesive or cement, such as silicate of soda, to constitute a relatively rigid unitary composite sheet.

Fig. 2 illustrates a vertical section of the composite wall board of Fig. 1. 70

Fig. 3 illustrates a composite wall board in which each and all of the single ply sheets, numbered 10 to 14, inclusive, and united to form the composite board, are formed from wood pulp or embody a percentage of wood pulp manufactured from steamed or boiled hard wood. While this construction may have certain advantages over the construction of Fig. 1, it, nevertheless, has this disadvantage, viz: The completed board is of the brown color characteristic of wood pulp manufactured from hard wood after steaming or boiling, while for many purposes a much lighter color is desirable as, for instance, the grayish-white 85 color characteristic of wood pulp manufactured from soft wood. For the purpose of giving the desired color to the external surfaces of the wall board, while utilizing as much hard wood pulp as possible in the 90 completed board, I have disclosed the construction of Fig. 4.

This figure illustrates a composite board in which the three central sheets or plies consist of or comprise wood pulp manufactured from steamed or boiled hard wood, while the outer sheets, 6 and 7, each consist of a single ply embodying an outer layer or series of layers —8— formed of wood pulp made from soft wood or other material, and an inner layer or series of layers —9— formed of or embodying wood pulp manufactured from steamed or boiled hard wood. These outer sheets, 6 and 7, are manufactured on the usual and well known board 100 machine with as many cylinders as desired running on pulp produced from steamed or boiled hard wood, and one or more cylinders running on pulp produced from soft wood or other material, producing a single ply or sheet consisting of a plurality of layers in the usual manner. 105

It will be understood that a percentage of soft wood pulp or paper stock pulp or other material may be added to the hard 110 wood pulp during the beating or mixing process with perhaps somewhat less advantageous results and that the composite board may be formed of any desired number of plies or laminations and that such laminations, plies or sheets may be secured together in any suitable manner and that each sheet may consist of, or comprise, any desired percentage of wood pulp manufactured from hard wood cooked by the steaming or boiling 120 process, and that various modifications may be made in the details of the process and the product all without departing from the invention as set forth in the appended 125 claims. 130

**What I claim is:—**

1. A laminated board suitable for wall board or other purposes, the center plies of which include wood pulp manufactured from ground cooked hard wood and the outer plies of which include pulp manufactured from other material.
2. A laminated board having a central ply consisting of ground, cooked, hard wood, and two facing plies consisting of pulp made from different material.
3. Wall board comprising a sheet of ground, cooked, hard wood pulp faced on both sides with soft wood pulp.
4. Wall board comprising a relatively rigid layer of ground, cooked, hard wood

pulp having a less rigid facing of soft wood pulp.

5. A laminated board suitable for wall board or other purposes, comprising a relatively rigid layer consisting substantially of wood pulp manufactured from ground, cooked hard wood, and a less rigid facing layer consisting of pulp manufactured from other material.

In witness whereof I have hereunto set my hand this 16th day of October, 1919.

HARRY S. LEWIS.

**Witnesses:**

H. E. CHASE,  
E. A. THOMPSON.